

## UNITED STATES PATENT OFFICE

2,167,906

## PROCESS OF CASTING

Carl Piel, Solingen, Germany

No Drawing. Application January 25, 1937, Serial No. 122,211. In Germany January 27, 1936

2 Claims. (Cl. 22—212)

This invention relates to processes of casting and, more particularly, to processes of casting carried out by means of metal or chill-moulds.

The permanent moulds or chills that have heretofore been used in processes of this kind had consisted of iron, steel or other metals, said moulds or chills having frequently been provided, prior to carrying out the casting process or subsequent to a number of such processes, with a coating at their interior wall, which coating consisted of insulating materials dissolved in water. A coating of this kind is intended to prevent the formation of a chemical compound between the metal of the chill-mould with the metal to be cast therein. This coating, which had heretofore been applied to the mould by hand, for instance by means of a brush, swab or the like, is connected with the disadvantage, that the surface of the chill is liable to become of uneven conformation, which will greatly impair the appearance and exactness of the castings. The castings, therefore, can frequently not be used without an expensive subsequent operation of finishing. A further disadvantage arises in connection with the making of proper castings from heavy metals, especially from alloys on copper basis with zinc, tin, lead or similar constituents, by means of metal chills, this disadvantage consisting therein that owing to the imperviousness of the chill the flow of liquid metal within the mould will be irregular, with the result that flaws or bubbles are liable to be present in the completed casting. This naturally renders it difficult, if not impossible, to make proper castings.

All aforementioned disadvantages, now, are successfully avoided by my invention by immersing the chill in heated condition into a water-bath prior to each process of casting. This bath according to my invention further contains powdered, insulating materials, such as minerals or oxides, in evenly distributed and floating condition therein. Such materials may advantageously consist of materials that are unable to form gases, for instance of graphite, chalk, clay, oxide of aluminum, argillaceous earth, oxide of zinc, oxide of lead, talc, sand and other kinds of earth having similar properties.

The chill-mould according to my invention is further heated to a temperature of about 400° C. or more causing red incandescence of the mould and thereupon chilled in said water-bath containing in fine distribution the aforementioned powdered materials. By immersing the mould in this highly heated condition into said bath the temperature of the latter will be raised

to boiling temperature causing the insulating coating which had remained in the mould from the preceding process of casting in wholly or partly destroyed condition to be separated from said mould. After said mould has been cooled down in said bath, the insulating materials contained in the latter will deposit on the surfaces of the mould, thus renewing the insulating coating that had remained in the mould in partly or wholly destroyed condition in the form of a perfect and uniform coating. This renewing of the coating due to the drop of temperature of the mould when being immersed in the bath, is connected in case of casting alloys of heavy metals containing lead, zinc or tin with the further advantage that the oxides formed during casting in the mould will deposit on said coating which consists of an amorphous non-coherent mass.

In this manner said oxides are prevented against depositing on the surface of the mould itself thus protecting the latter against injury, said oxides being separated from the mould when being immersed in the boiling bath subsequent to each previous process of casting. A separation of the deposits of oxides by means of special implements, such as brushes or the like, is not necessary in the present case in order to obtain smooth surfaces on the castings.

The thickness of the insulating coating so produced on the mould by immersion depends upon the amount of powdered materials contained in the bath. These powdered materials will produce, subsequent to evaporation of the water of the bath, an insulating coating of even thickness and of a uniformity that cannot be attained otherwise. By my present process the mould, as regards the metal to be cast, will be given properties nearly as favorable as in case of using a mould consisting of sand, for the metal while being cast will flow instead of over the rigid and impervious metal-wall of the mould over said insulating coating formed on the latter by said minerals. As a result of this the metal while being cast will properly and completely fill the mould and move therein in a quiet and even flow, effectively preventing any formation of flaws, bubbles or the like in the completed casting.

The insulating coating formed by said minerals does not need to present a fully coherent surface. It may even be of advantage if small interstices are present in said insulating coating, as said interstices will enclose small amounts of air forming part of the insulating coating, the presence of such air having a favorable effect upon

the process of casting. In the present case, during casting there is produced a pressure in the mould, this pressure being due, firstly, to the gravity of the metal present in the mould and secondly to the still more effective action of the air cushion which is being formed between the flowing metal and the insulating coating, especially if the latter is not fully coherent. These small quantities of air now will expand by action of the high temperature of the metal flowing in the mould and in consequence of this, in the latter there will be produced a pressure forcing the metal while being cast into the tiniest corners and angles of the mould, this pressure essentially assisting in the production of sharp-edged and exactly formed castings that may be used without further finishing. The quality of the castings, especially in case of copper alloy castings, may further be improved by adding small quantities of earth-metals, silicon or manganese, to the metal prior to the casting. These admixtures have the effect of producing a thin layer of oxide during casting of the metal into the mould which had been chilled in the bath by previous immersion thereinto, the formation of this thin layer of oxide being due to sudden cooling. This layer of oxide is of the form of a film that is transparent and coherent in itself and inseparably connected with the casting as well as surrounding the latter on all sides thereof. By this, the wall of the mould will be insulated against the metal cast thereinto as the formed thin film consists of a mass which is chemically immune, with the result of considerably lengthening the life-time of the mould. Besides, by this procedure the castings will be given a smooth surface of metallic shine giving the last finish to the casting and, in addition to this, enhancing its resistivity against corrosion, the said thin film effectively protecting the casting against any outer influence.

The aforementioned sudden cooling or chilling of the metal in the mould will cause a condensation of the admixtures contained in the melted mass, said admixtures depositing on the surface of the casting and turning into oxides by action of the high temperature. The high tensions and pressures produced by sudden cooling or chilling of the metal as well as the small quantity of oxygen contained in said thin layer of oxide will have the effect of transforming said layer into a certain structure which is quite different from that produced with normal oxides consisting of an amorphous mass and forming a layer of considerable thickness. Such oxides are being produced, for instance, by casting in dry sand in which case there is slow cooling and unimpeded access of oxygen from the air during the long period of cooling. In contradistinction to this, the low temperature of the mould due to immersion of the latter into the bath prior to each process of casting will produce an extremely thin layer consisting of a precious oxide covering the surface of the casting in the form of a fully uniform and transparent film.

When commencing the casting, the mould is preferably pre-heated to the required temperature, while for subsequent casting the mould is cooled or chilled by immersion in the bath down to the required temperature, in which case the mould may remain in the bath, if desired for some longer time eventually for several minutes, until it has assumed the proper temperature.

The temperature of the mould prior to each casting process is dependent upon the composi-

tion of the alloy to be cast. If brass or another copper-alloy containing tin or zinc is used for casting, the temperature of the mould must be about 100° C. so that a drop of temperature amounting to about 900° C. will arise between the copper-alloy which is cast at about 1000° C. into the mould and the wall of the latter. In case the copper-alloy includes constituents which only difficultly alloy with the copper, such as for instance lead, a somewhat lower temperature will be required for the mould in order to effect the heavy chilling of the metal necessary for the formation of said film and for producing a uniform covering on the casting. On the bases of experiments I have found that the most favorable temperature of the mould amounts in this case to about from 40 to 80° C.

In case of copper-alloys containing about from 12 to 15 percent of lead, these alloys being of especial importance as a substitute for tin-bronzes, it is advisable to further chill the casting in still hot condition after completion of the process by dropping the casting from the mould into a water-bath. This further chilling will assist the formation of said film and effectively prevent the separation of lead. In this manner high-grade castings may also be made from copper-alloys having a high content of lead or other constituents that only difficultly alloy with copper. Such copper-alloys could heretofore hardly be cast in chilled moulds, while the castings obtained according to my present process may be used without any further finishing that is as a finished product produced solely by casting.

The chilling of the metal moulds which I propose in accordance with my invention by immersing the mould into a bath, besides the formation of said film on the surface of the casting, is further connected with the advantage that the casting obtained by the new process will be of a finer structure, especially if subsequent to the process the casting is subject to further chilling.

To the copper-alloy there may be added, for instance immediately before the process of casting, a small quantity, about one percent, of aluminum which forms a solid solution in copper. As a result of the sudden cooling or chilling during the casting of the metal in the mold, which has been chilled below 150° C., the aluminum combines but incompletely, at the top surface, with the oxygen of the atmosphere. Thus an oxide is formed which is poor in oxygen and possesses entirely different characteristics from ordinary aluminum oxide. The so produced thin layer of non-corrosive aluminum oxide owing to the rapidity of chilling will be cooled down so effectively that a further diffusion of oxygen into the casting, that is through the film thereon, is rendered impossible, the same as an exit of the aluminum atom from the oxide molecule, as the velocity of diffusion has yet become too small owing to the cooling which has taken place in the meanwhile.

In principally like manner a uniform film may be produced all over the surface of the casting, if other film-forming metals such as silicon, manganese or the like are added to the copper-alloy which together with such additions is now cast into the chilled or only little pre-heated mould.

The quantity of additional metal necessary for the formation of the film is very small and amounts in general only to about one percent of the constituents of the alloy. It is of especial advantage in this case that the small admixture

of metals sufficient for the formation of the film does not impair the properties and the character of the alloy in the casting. The presence of the aforementioned admixed metals, therefore, can 5 hardly be ascertained.

My present invention, besides for copper-alloys, is also of importance and advantage for other difficultly melting metals other than iron, such as for instance silver; in this case also a protective film may be provided on the casting rendering it possible to use the same without any further finishing.

I claim:

1. A process of making copper alloy castings in metal molds, which process comprises the steps of immersing the mold into a water bath containing powdered insulating material finely dispersed therein until the mold has been chilled to a temperature below 80° C. and a thin insulating 10 coating has been formed on its inner surface, and then casting into said mold an alloy of copper with between 10 and 15 percent lead and about one percent of a substance selected from the 20 group consisting of earth metals, silicon and manganese.

2. A process of making copper alloy castings

in a metal mold in continuous succession, which process comprises the steps of immersing the mold into a water bath containing powdered insulating material until the mold has been chilled and a thin insulating coating has been formed on its inner surface, casting into said mold an alloy containing a copper base and a small quantity of a metal selected from the group consisting of earth metals, silicon and manganese, whereby the mold is heated to red incandescence and said insulating coating is at least partly destroyed by being converted into an amorphous non-coherent mass on which some of the metal oxides formed during the casting are deposited, removing the finished casting from the mold, and reinserting the latter while still red hot into said bath, whereby the bath first comes to a boil which assists in separating the residua of said insulating coating and said oxide deposits from the walls of the mold and then the mold is chilled to the desired temperature while the powdered insulating materials contained in said bath form a new and complete insulating lining, whereupon the mold is ready for another casting.

CARL PIEL. 25